

# United States Patent [19]

Gingello et al.

[11] Patent Number: 5,061,595

[45] Date of Patent: Oct. 29, 1991

[54] CONTACT FILM FOR USE IN GRAPHIC ARTS WITH TWO OVERCOAT LAYERS

[75] Inventors: Anthony D. Gingello, Rochester; David F. Jennings, Penfield; Richard D. Lucitte, Holcomb; Hermano P. Rocha, Rochester, all of N.Y.

[73] Assignee: Eastman Kodak Company, Rochester, N.Y.

[21] Appl. No.: 590,707

[22] Filed: Sep. 24, 1990

[51] Int. Cl.<sup>5</sup> G03C 1/36; G03C 1/02

[52] U.S. Cl. 430/264; 430/523; 430/531; 430/539; 430/950; 430/961; 430/606

[58] Field of Search 430/264, 539, 950, 961, 430/531, 523

## [56] References Cited

### U.S. PATENT DOCUMENTS

- |           |         |                  |         |
|-----------|---------|------------------|---------|
| 4,232,117 | 3/1980  | Naoi et al.      | 430/539 |
| 4,343,873 | 4/1982  | Sasaoka          | 430/1   |
| 4,777,113 | 8/1988  | Inoue et al.     | 430/264 |
| 4,818,659 | 11/1989 | Takahashi et al. | 430/264 |
| 4,847,180 | 7/1989  | Miyata et al.    | 430/264 |
| 4,855,219 | 1/1989  | Bagchi et al.    | 430/496 |
| 4,914,012 | 3/1990  | Kawai            | 430/536 |

4,933,272 6/1990 McDugle et al. .... 430/567

Primary Examiner—Richard L. Schilling  
Attorney, Agent, or Firm—Alfred P. Lorenzo

[57]

## ABSTRACT

A high-contrast room-light-handleable black-and-white silver halide photographic film especially adapted for use as a dry-dot-etchable contact film in the graphic arts is comprised of a support having in order on one side thereof (1) a radiation-sensitive layer comprising silver halide grains, a hydrophilic colloid and a polymer latex, (2) an interlayer comprising a hydrophilic colloid and a polymer latex, and (3) an overcoat layer comprising a hydrophilic colloid, a matting agent and a light-scattering agent, wherein the interlayer has a refractive index in the range of from about 1.4 to about 1.7 and a thickness which is in the range of from about 0.5 to about 5 microns and is at least twice that of the overcoat layer. The combination of the light-scattering agent in the overcoat layer and the thick interlayer facilitates optical spreading of the image during contact exposure, and thereby enhances the performance of the contact film in use with multi-layer originals and in processes of dry dot etching.

15 Claims, No Drawings

## CONTACT FILM FOR USE IN GRAPHIC ARTS WITH TWO OVERCOAT LAYERS

### FIELD OF THE INVENTION

This invention relates in general to photography and in particular to black-and-white silver halide photographic films. More specifically, this invention relates to high-contrast black-and-white silver halide photographic films which are adapted for room-light handling and especially useful in the field of graphic arts.

### BACKGROUND OF THE INVENTION

An important class of photographic films are black-and-white silver halide films intended to be used for contact exposures in the field of graphic arts. Such films require a high degree of dimensional stability as well as a surface which is non-tacky, and has a suitable degree of roughness to facilitate rapid vacuum draw-down during contact exposure. Advantageously, these films are relatively low in photographic speed so that they can be used under bright safelight or even ordinary room-light conditions. To facilitate handling in use, it is highly desirable that the front and back surfaces of the contact film be readily distinguishable by the user.

An additional highly desirable property for the aforesaid graphic arts contact films is the ability to optically spread the image during contact exposure. Thus, for example, in employing dot image originals, it is desirable to be able to regulate the degree of dot growth that occurs on contact exposure. Also, the original which is to be exposed in the contact exposure process can, in some instances, be a multi-layer original, that is, an original in which two or more elements have been stacked together as an assembly. Such a multi-layer assembly can include both line image originals and dot image originals. The ability to optically spread the image during exposure is critically important in handling such stacked originals in a single exposure process. In particular, optical spreading can improve the image quality of characters produced from originals which are out of contact with the contact film.

Optical image spread is distinguished from chemical image spread which involves infectious imagewise development of unexposed photographic silver halide grains in close proximity to exposed photographic silver halide grains. Chemical image spread is achieved by incorporation of a nucleating agent in either the film or the developing solution. A given system can employ either optical image spread or chemical image spread or both.

To facilitate optical spreading of an image during contact exposure, it is important that the silver halide emulsion layer of the contact film be widely spaced from the surface of the contact film that comes into 55 face-to-face contact with the original, such surface typically being the surface of a protective overcoat layer which serves as the outermost layer of the film.

It is increasingly common in the graphic arts to employ a computer assisted "dry dot etching" process in 60 making color corrections to halftone separations. The process can be carried out without the use of masks for color correction of an entire separation, or it can be done with hand-cut masks or photographic masks for local color corrections. Techniques used in dry dot etching vary from shop to shop, but all depend on the ability of a contact or duplicating film to change dot size with overexposure (overexposure meaning an expo-

sure greater than that necessary to produce dot-for-dot reproduction in the midtone dot values). Generally, the dot-change exposure technique starts with a dot-for-dot exposure and adds a "bump", or additional, exposure to produce the desired change in dot value. This "bump" exposure may be confined to a localized area of the subject by masking, or it may be combined with the dot-for-dot exposure to make an overall change to the separation. Contact films which are best suited for use in dry dot etching are those that provide a high degree of optical spread.

It is exceedingly difficult to incorporate in a photographic film all of the properties that are desirable for use as a contact exposure film in the graphic arts. Thus, for example, the use of a very thick overcoat layer to provide the desired spacing between the surface of the film and the silver halide emulsion layer is impractical, since it adversely affects dimensional stability. To improve dimensional stability, a polymer latex can be incorporated in the overcoat layer, but this tends to render the surface undesirably tacky. Also, if the overall thickness of the hydrophilic layers, including the emulsion layer and overcoat layer, becomes too great, the diffusion of developing agents and fixing agents to the emulsion layer will be impeded and the time required for development and fixing will be excessive. Yet another problem will be the prolonged drying period needed to dry the processed film.

The present invention is directed to a novel contact film for use in the graphic arts which effectively overcomes all of the above problems and combines a wide variety of desired features in a single film.

### SUMMARY OF THE INVENTION

In accordance with this invention, a high-contrast room-light-handleable black-and-white silver halide photographic film especially adapted for use as a dry-dot-etchable contact film in the graphic arts is comprised of a support having in order on one side thereof (1) a radiation-sensitive layer comprising silver halide grains, a hydrophilic colloid and a polymer latex, (2) an interlayer comprising a hydrophilic colloid and a polymer latex, and (3) an overcoat layer comprising a hydrophilic colloid, a matting agent and a light-scattering agent, wherein the interlayer has a refractive index in the range of from about 1.4 to about 1.7 and a thickness which is in the range of from about 0.5 to about 5 microns and is at least twice that of the overcoat layer.

The novel photographic film of this invention has good dimensional stability characteristics and a non-tacky matte surface which facilitates rapid vacuum draw-down during contact exposure. It is room-light-handleable and capable of producing images of the high contrast desired in the graphic arts. The overcoat layer is characterized by a degree of haze sufficient to enable the user to readily distinguish between the front and back surfaces of the film. The overall thickness of the combination of emulsion layer, interlayer and overcoat layer is such that development and fixing can be carried out in suitably short periods of time. The combination of the light-scattering agent in the overcoat layer and the thick interlayer facilitates optical spreading of the image during contact exposure, and thereby enhances the performance of the contact film in use with multi-layer originals and in processes of dry dot etching.

DESCRIPTION OF THE PREFERRED  
EMBODIMENTS

The contact film of this invention can utilize any of the polymeric film supports known for use in the photographic arts. Typical of useful polymeric film supports are films of cellulose nitrate and cellulose esters such as cellulose triacetate and diacetate, polystyrene, polyamides, homo- and co-polymers of vinyl chloride, poly(vinylacetate), polycarbonate, homo and co-polymers of olefins, such as polyethylene and polypropylene and polyesters of dibasic aromatic carboxylic acids with divalent alcohols, such as poly(ethylene terephthalate).

Polyester films, such as films of polyethylene terephthalate, have many advantageous properties, such as excellent strength and dimensional stability, which render them especially advantageous for use as supports in the present invention.

The polyester film supports which can be advantageously employed in this invention are well known and widely used materials. Such film supports are typically prepared from high molecular weight polyesters derived by condensing a dihydric alcohol with a dibasic saturated fatty carboxylic acid or derivatives thereof. Suitable dihydric alcohols for use in preparing polyesters are well known in the art and include any glycol, wherein the hydroxyl groups are on the terminal carbon atom and contain from 2 to 12 carbon atoms such as, for example, ethylene glycol, propylene glycol, trimethylene glycol, hexamethylene glycol, decamethylene glycol, dodecamethylene glycol, and 1,4-cyclohexane dimethanol. Dibasic acids that can be employed in preparing polyesters are well known in the art and include those dibasic acids containing from 2 to 16 carbon atoms. Specific examples of suitable dibasic acids include adipic acid, sebacic acids, isophthalic acid, and terephthalic acid. The alkyl esters of the above-enumerated acids can also be employed satisfactorily. Other suitable dihydric alcohols and dibasic acids that can be employed in preparing polyesters from which sheeting can be prepared are described in J. W. Wellman, U.S. Pat. No. 2,720,503, issued Oct. 11, 1955.

Specific preferred examples of polyester resins which, in the form of sheeting, can be used in this invention are poly(ethylene terephthalate), poly(cyclohexane 1,4-dimethylene terephthalate), and the polyester derived by reacting 0.83 mol of dimethyl terephthalate, 0.17 mol of dimethyl isophthalate and at least one mol of 1,4-cyclohexanedimethanol. U.S. Pat. No. 2,901,466 discloses polyesters prepared from 1,4-cyclohexanedimethanol and their method of preparation.

The thickness of the polyester sheet material employed in carrying out this invention is not critical. For example, polyester sheeting of a thickness of from about 0.05 to about 0.25 millimeters can be employed with satisfactory results.

In a typical process for the manufacture of a polyester photographic film support, the polyester is melt extruded through a slit die, quenched to the amorphous state, oriented by transverse and longitudinal stretching, and heat set under dimensional restraint. In addition to being directionally oriented and heat set, the polyester film can also be subjected to a subsequent heat relax treatment to provide still further improvement in dimensional stability and surface smoothness.

In the contact film described herein, the layer overlying the support is a negative-working emulsion layer comprising a hydrophilic colloid, a polymer latex and

radiation-sensitive silver halide grains capable of forming a surface latent image. One or more subbing layers which function to enhance the bonding of the silver halide emulsion layer to the support are also advantageously included in the film.

The photographic films of this invention are high contrast films with the particular contrast value, as indicated by gamma ( $\gamma$ ), depending on the type of emulsion employed. Gamma is a measure of contrast that is well-known in the art as described, for example, in James, *The Theory of the Photographic Process*, 4th Ed., 502, MacMillan Publishing Co., 1977.

The useful silver halide emulsions include silver chloride, silver bromide, silver chlorobromide, silver bromoiodide, silver chloroiodide and silver chlorobromoiodide emulsions.

The silver halide grains useful in the practice of the invention may be of any known configuration, including regular octahedral, cubic, or tabular grains, as described, for example, in *Research Disclosure*, Item 17643, December 1978, Section I, and *Research Disclosure*, Item 22534, January, 1983. The silver halide grains preferably have a mean grain size of not greater than about  $0.7\mu$  and more preferably of about  $0.4\mu$  or less. As is recognized in the art, higher contrasts can be achieved by using relatively monodispersed emulsions, particularly when larger grain size emulsions are employed. As used herein, the term "monodispersed" means that the emulsion has a coefficient of variation of less than about 20%. For the highest levels of contrast, the coefficient of variation is preferably less than about 10%. As used herein, the term "coefficient of variation" is defined as 100 times the standard deviation of the grain diameter divided by the mean grain diameter.

The amount of silver in the contact film of this invention is preferably in the range of from about 0.01 to about 0.05 moles per square meter.

In the contact film of this invention, room-light-handleable characteristics can be achieved by any of several procedures. For example, absorbing layers can be used to screen undesired radiation from coming into contact with the silver halide emulsion layer. Filter dyes can be used to achieve this objective. Alternatively, an absorbing layer comprising silver halide grains of reduced photosensitivity can be employed. Such layers are described in copending commonly assigned U.S. patent application Ser. No. 475,542, entitled "Absorbing Layer For Photographic Speed Reduction", filed by A. D. Gingello et al on Feb. 6, 1990, the disclosure of which is incorporated herein by reference. As a further alternative, a doping agent can be incorporated in the silver halide grains of the radiation-sensitive silver halide emulsion layer in an amount effective to reduce the speed sufficiently to provide the desired room-light-handleable characteristics. Use of such doping agents is a preferred technique in the present invention.

McDugle et al, U.S. Pat. No. 4,933,272 issued June 12, 1990, the disclosure of which is incorporated herein by reference, discloses silver halide emulsions comprised of radiation sensitive silver halide grains exhibiting a face centered cubic crystal lattice structure internally containing a nitrosyl or thionitrosyl coordination ligand and a transition metal chosen from groups 5 to 10 inclusive of the periodic table of elements. These emulsions are preferred for use in the contact film of this invention.

In accordance with the aforesaid U.S. Pat. No. 4,933,272, the dopants contained within the silver halide grains are transition metal coordination complexes which contain one or more nitrosyl or thionitrosyl ligands. These ligands have the formula:



where X is oxygen in the case of nitrosyl ligands and sulfur in the case of thionitrosyl ligands.

Preferred dopants utilized in this invention are transition metal coordination complexes having the formula:



wherein:

M is a ruthenium, rhenium, chromium, osmium or iridium transition metal;  
X is oxygen or sulfur;  
L is a ligand; and  
n is -1, -2, or -3.

As in the aforesaid U.S. Pat. No. 4,933,272, all references herein to periods and groups within the periodic table of elements are based on the format of the periodic table adopted by the American Chemical Society and published in the *Chemical and Engineering News*, Feb. 4, 1985, p. 26. In this form the prior numbering of the periods was retained, but the Roman numeral numbering of groups and designations of A and B groups (having opposite meanings in the U.S. and Europe) was replaced by a simple left to right 1 through 18 numbering of the groups.

Silver halide emulsions also contain a hydrophilic colloid that serves as a binder or vehicle. The proportion of hydrophilic colloid can be widely varied, but typically is within the range of from about 20 to 250 g/mole silver halide. The presence of excessive levels of hydrophilic colloid can reduce maximum image density and, consequently, contrast. Thus, for  $\gamma$  values of 10 or more, the vehicle is preferably present at a level of less than 200 g/mole silver halide.

The hydrophilic colloid is preferably gelatin, but many other suitable hydrophilic colloids are also known to the photographic art and can be used alone or in combination with gelatin. Suitable hydrophilic colloids include naturally occurring substances such as proteins, protein derivatives, cellulose derivatives—e.g., cellulose esters, gelatin—e.g., alkali-treated gelatin (cattle bone or hide gelatin) or acid-treated gelatin (pigskin gelatin), gelatin derivatives—e.g., acetylated gelatin, phthalated gelatin and the like, polysaccharides such as dextran, gum arabic, zein, casein, pectin, collagen derivatives, collodion, agar-agar, arrowroot, albumin, and the like.

In addition to the hydrophilic colloid and the silver halide grains, the radiation-sensitive silver halide emulsion layer employed in the contact film of this invention includes a polymer latex which serves to improve the dimensional stability of the film. Polymers useable in latex form for this purpose are very well known in the photographic art. The requirements for such a polymer latex are (1) that it not interact with the hydrophilic colloid such that normal coating of the emulsion layer is not possible, (2) that it have optical properties, i.e., refractive index, similar to that of the hydrophilic colloid, and (3) that it have a glass transition temperature

such that it is plastic at room temperature. Preferably, the glass transition temperature is below 20° C.

The polymer latex useful in the present invention is an aqueous dispersion of a water-insoluble polymer. It is incorporated in the emulsion layer in an amount that is typically in the range of from about 0.2 to about 1.5 parts per part by weight of the hydrophilic colloid.

The synthetic polymeric latex materials referred to herein are generally polymeric materials which are relatively insoluble in water compared to water-soluble polymers, but have sufficient water solubility to form colloidal suspensions of small polymeric micelles. Typical latex polymeric materials can be made by rapid copolymerization with vigorous agitation in a liquid carrier of at least one monomer which would form a hydrophobic homopolymer and at least one monomer which would form a hydrophilic homopolymer. In certain preferred embodiments, from about 1 to about 30 percent, by weight, of units of monomer containing the water-solubilizing group is present in the copolymer product. Copolymers prepared by this method and analogous methods provide discrete micelles of the copolymer which have low viscosities in aqueous suspensions. Typical useful copolymers include interpolymers of acrylic esters and sulfoesters as disclosed in Dykstra, U.S. Pat. No. 3,411,911 issued Nov. 19, 1968, interpolymers of acrylic esters and sulfobetains as described in Dykstra and Whiteley, U.S. Pat. No. 3,411,912 issued Nov. 19, 1968, interpolymers of alkyl acrylates and acrylic acids as disclosed in Ream and Fowler, U.S. Pat. No. 3,287,289 issued Nov. 22, 1966, interpolymers of vinyl acetate, alkyl acrylates and acrylic acids as disclosed in Corey, U.S. Pat. No. 3,296,169, and interpolymers as disclosed in Smith, U.S. Pat. No. 3,459,790 issued Aug. 5, 1969. Polymeric latex materials can also be made by rapid polymerization with vigorous agitation of hydrophobic polymers when polymerized in the presence of high concentrations of surfactants which contain water-solubilizing groups. The surfactants are apparently entrained in the micelle and the solubilizing group of the surfactant provides sufficient compatibility with aqueous liquids to provide a dispersion very much like a soap. Generally good latex materials are also disclosed in Nottorf, U.S. Pat. No. 3,142,568 issued July 28, 1964; White, U.S. Pat. No. 3,193,386 issued July 6, 1965; Houck et al., U.S. Pat. No. 3,062,674 issued Nov. 6, 1962; and Houck et al., U.S. Pat. No. 3,220,844 issued Nov. 30, 1965.

The synthetic polymeric latex materials are generally polymerized in a manner to produce micelles of about 1.0 micron average diameter or smaller to be highly useful in photographic emulsions and preferably the discrete micelles are less than 0.3 micron in average diameter. Generally, the micelles can be observed by photomicrographs when incorporated in gelatino emulsions, however, it is understood that some coalescing can occur when the emulsions are coated and dried.

In one embodiment, the latex polymers which can be used according to this invention are acrylic interpolymers, i.e., those interpolymers prepared from polymerizable acrylic monomers containing the characteristic acrylic group



Such polymers are conveniently prepared by the interpolymerization of an acrylic monomer with at least one dissimilar monomer which can be another acrylic monomer or some other different polymerizable ethylenically unsaturated monomer. It is, of course, understood that the acrylic interpolymers employed in the practice of this invention are compatible with gelatin and have a  $T_g$  (glass transition temperature) of less than 20° C. ( $T_g$  can be calculated by differential thermal analysis as disclosed in "Techniques and Methods of Polymer Evaluation", Vol. 1, Marcel Dekker, Inc., N.Y., 1966).

A particularly preferred polymer latex for use in the silver halide emulsion layer is poly(methylacrylate-co-2-acrylamido-2-methyl propane sulfonic acid) which is comprised of repeating units of the formula:



The thickness of the radiation-sensitive silver halide emulsion layer in the improved contact film of this invention is typically in the range of from about 1 to 35 about 9 microns, and more preferably in the range of from about 2 to about 4 microns.

The term "room-light-handleable", as used herein, is intended to denote that the film can be exposed to a light level of 200 lux for several minutes without a significant loss in maximum density. Typically, such materials require on the order of 10,000 ergs per square centimeter of  $D_{min}$  exposure.

In the improved contact film of this invention, an interlayer is positioned between the silver halide emulsion layer and the overcoat layer. The interlayer is intended to serve primarily as a spacing layer. It has a thickness of at least twice, and more preferably at least three times, that of the overcoat layer.

Image manipulation, which has been briefly referred to hereinabove, is a critical consideration in regard to the structural arrangement of the layers in the novel photographic films described herein and particularly in regard to the thickness and properties of the interlayer. In many types of photographic films, it is highly advantageous for the spread function to be small because this enhances image sharpness and thereby enables the preparation of high quality enlargements. Most contact films used in the field of graphic arts are comprised of very small silver halide grains in order to provide low speeds and, as a consequence, the spread function tends to be small. However, in such graphic arts films, the impression of quality is derived from the acutance at edges, for both dots and lines, which is driven by sensitometric curve shape, and thus spread function is not important in regard to image quality. It is, however, very important in regard to image manipulation; the term "image manipulation" referring to the ability to optically

change the size of halftone dots and lines by reducing or increasing the exposure given.

Image manipulation is extremely important in adjustment of color reproduction in the final print as well as for tonal changes. Small spread functions are the enemy of image manipulation. This is clear upon considering the mechanism of increasing the area of a halftone dot solely by use of exposure. The image space of a halftone dot or line edge is the convolution of the original image with the spread function of the imaging system. In a contact printing situation, it is almost entirely the spread function of the emulsion. Thus, graphic arts contact films pose a dilemma. The necessary use of fine grain emulsions provides small spread functions, whereas large spread functions are needed to effectively manipulate the images.

In the novel photographic films of this invention, the interlayer serves as an efficient means to degrade the emulsion spread function in a contact printing environment. The interlayer provides a physical space between the image and the radiation-sensitive emulsion and this space enhances lateral spreading of the exposing radiation and creates a softer image edge profile.

To achieve an effective degree of optical spread, it is necessary that the interlayer have a refractive index in the range of from about 1.4 to about 1.7, and more preferably in the range of from about 1.55 to about 1.65.

The interlayer is comprised of a mixture of a polymer latex and a hydrophilic colloid. The purpose of the polymer latex is to impart the necessary dimensional stability to the film and for this purpose, it is employed in an amount of from about 0.2 to about 1.5 parts per part by weight of the hydrophilic colloid. The hydrophilic colloid incorporated in the interlayer can be selected from among those described above as being useful in the emulsion layer and can be the same or different than the particular hydrophilic colloid used in the emulsion layer. Most preferably, the hydrophilic colloid in the interlayer is gelatin. The polymer latex incorporated in the interlayer can be selected from among those described above as being useful in the emulsion layer and can be the same or different than the polymer latex used in the emulsion layer. Most preferably, the polymer latex in the interlayer is poly(methylacrylate-co-2-acrylamido-2-methylpropane sulfonic acid).

The thickness of the interlayer is typically in the range of from about 0.5 to about 5 microns, preferably in the range of from about 0.8 to about 3.5 microns, and most preferably in the range of from about 1.7 to about 3 microns.

The overcoat layer in the improved contact film of this invention is comprised of a hydrophilic colloid, a matting agent and a light-scattering agent. The hydrophilic colloid can be selected from among those described above as being useful in the emulsion layer and the interlayer and can be the same or different than the hydrophilic colloid used in those layers. Most preferably, the hydrophilic colloid in the overcoat layer is gelatin.

The overcoat layer comprises discrete solid particles of a matting agent typically having an average particle size in the range of from about 1 to about 5 microns and preferably in the range of from about 2 to about 4 microns. The matting agent is typically employed in an amount of from about 0.02 to about 1 part per part by weight of the hydrophilic colloid. Either organic or inorganic matting agents can be used. Examples of organic matting agents are particles, often in the form of

beads, of polymers such as polymeric esters of acrylic and methacrylic acid, e.g., poly(methylmethacrylate), cellulose esters such as cellulose acetate propionate, cellulose ethers, ethyl cellulose, polyvinyl resins such as poly(vinyl acetate), styrene polymers and copolymers, and the like. Examples of inorganic matting agents are particles of glass, silicon dioxide, titanium dioxide, magnesium oxide, aluminum oxide, barium sulfate, calcium carbonate, and the like. Matting agents and the way they are used are further described in U.S. Pat. Nos. 3,411,907 and 3,754,924.

The overcoat layer also comprises discrete solid particles of a light-scattering agent typically having an average particle size in the range of from about 0.1 to about 5 microns, and preferably in the range of from about 0.5 to about 1.5 microns. The light-scattering agent is typically employed in an amount of from about 0.02 to about 1 part per part by weight of the hydrophilic colloid.

Either organic light-scattering agents, such as particles of polymethylmethacrylate, or inorganic light-scattering agents, such as silver halides, calcium carbonate, or silicon dioxide, can be used. The light-scattering agent used in this invention has particles large enough to scatter visible light and therefore to cause the formation of haze in the film. This is advantageous in enabling the user of the film to readily distinguish between the front and back surfaces. The amount of scattering is affected by the size and shape of the particles and by the difference between the refractive index of the particles and the medium.

The light-scattering agent in the overcoat layer enhances the degree of optical spread achieved during contact exposure and thereby enables the combined thickness of the emulsion layer, interlayer and overcoat layer to be kept below that at which dimensional stability would be seriously harmed or processing times would be unduly prolonged.

If desired, the same particles can be used in the overcoat layer to serve as both the matting agent and the light-scattering agent. For example, polymethylmethacrylate beads or silicon dioxide particles of suitable size can serve reasonably well in both capacities. It is preferred, however, to use different materials as the matting agent and the light-scattering agent, so that each can have optimum properties for its particular purpose. In particular, it is preferred to use polymethyl methacrylate beads with an average particle size of about 4 microns as the matting agent and silica particles with an average size of about 2 microns as the light-scattering agent.

Particles used as matting agents and light-scattering agents in the present invention can be of essentially any shape. Their size is typically defined in terms of mean diameter. Mean diameter of a particle is defined as the 55 diameter of a spherical particle of identical mass. Polymer particles that are in the form of spherical beads are preferred for use as matting agents.

The thickness of the overcoat layer is typically in the range of from about 0.2 to about 1 microns, preferably 60 in the range of from about 0.3 to about 0.6 microns and most preferably in the range of from about 0.35 to about 0.45 microns.

The side of the support opposite to the emulsion layer, typically is coated with an anti-halation layer 65 whose function is to prevent light that passes through the film support from being reflected into the image-forming layer and thereby causing an undesired spread-

ing of the image which is known as halation. The anti-halation layer may in turn be overcoated with another layer which serves as a protective outermost layer.

As lithographic-type photographic elements, the 5 films of this invention are preferably utilized (exposed and processed) as sheet films. As such, the films preferably have low curl (i.e., less than about 40 ANSI curl units at 21° C. and 15% relative humidity, using ANSI PH 1.29-1971, which calls for matching the curl of sample strips on a template of curves of varying radii to determine the radius of curvature and reporting the value of 100/R as the degree of curl where R is the radius of curvature in inches) and high dimensional stability (humidity coefficient, defined as % change in linear dimension divided by change in percent humidity over a 15-50% relative humidity range at 21° C., of less than about 0.0015).

The invention is further illustrated by the following example of its practice.

Element A, which is employed herein as a control, is comprised of a poly(ethylene terephthalate) film support, a silver halide emulsion layer overlying the film support, and a protective overcoat layer overlying the silver halide emulsion layer. On its opposite side, the film support is coated with an antihalation layer and a backing layer which overlies the antihalation layer. The silver halide emulsion layer is comprised of a negative-working silver chloride emulsion, doctored with 4-hydroxy-6-methyl-1,3,3a,7-tetraazaindene, containing silver halide grains capable of forming a surface latent image and has a dry thickness of 5 microns. The silver halide grains are described in Example 1 of U.S. Pat. No. 4,933,272, to which reference has been made hereinabove, except that they incorporate, as a dopant, the compound K<sub>2</sub>Ru(NO)Br<sub>5</sub>. The emulsion layer contains gelatin as a binder and a polymer latex, poly(methylacrylate-co-2-acrylamido-2-methyl propane sulfonic acid), is incorporated therein in an amount of 0.75 parts per part by weight of gelatin to improve dimensional stability. The overcoat layer is comprised of gelatin, polymethylmethacrylate beads with an average size of 4 microns in an amount of 0.02 parts per part by weight of gelatin, and silica with an average particle size of 2 microns in an amount of 0.025 parts per part by weight of gelatin, and has a dry thickness of 0.4 microns.

Element B, which is within the scope of the present invention, is identical to Element A, except that it additionally includes an interlayer interposed between the silver halide emulsion layer and the overcoat layer. The interlayer has a refractive index of 1.6 and a dry thickness of 2.1 microns and is composed of gelatin and 1 part, per part by weight of gelatin, of poly(methylacrylate-co-2-acrylamido-2-methyl propane sulfonic acid).

Each of elements A and B was exposed on a graphic arts contact printer unit developed for 33 seconds at 35° C. in KODAK Universal Rapid Access Developer and fixed for 33 seconds at 35° C. in Kodak RA-2000 fixing solution. Each element was evaluated to determine Multilayer Image Quality (MLIQ) and Dot Growth (DG) and the results obtained were as follows:

| Element | MLIQ<br>(% Dot Area) | DG<br>(% Dot Area/ΔLOG E) |
|---------|----------------------|---------------------------|
| A       | 71                   | 13.3                      |
| B       | 65                   | 19.0                      |

In the evaluation of MLIQ, Kanji characters, i.e. characters belonging to the Kanji system of writing that is used in Japan, are simultaneously exposed with scanner halftone dots in the E—E configuration. The measure of MLIQ reported above is the percent dot area of a 150 line per inch halftone positioned in the same layer as the Kanji characters. The value of this dot pattern, measured at the exposure where the E—E scanner halftone is acceptable, is a measure of the quality of the Kanji characters. The quality increases as the percent dot area decreases. In the data reported above, the change from an MLIQ of 71 to an MLIQ of 65 represents a significant improvement in quality attributable to the presence of the interlayer in Element B.

Dot growth refers to the rate of change of percent dot area with respect to log exposure, i.e. percent dot area divided by delta log E. Dot Growth is analogous to spread function in that an increase in Dot Growth represents an increase in spread function. As shown by the data above, the presence of the interlayer in Element B results in a substantial increase in dot growth and a corresponding significant improvement in the perceived quality of Kanji characters.

The invention has been described in detail with particular reference to preferred embodiments thereof, but it will be understood that variations and modifications can be effected within the spirit and scope of the invention.

We claim:

1. A high-contrast room-light-handleable black-and-white silver halide photographic film which is especially adapted for use as a dry-dot-etchable contact film in the graphic arts by its ability to optically spread an image during contact exposure; said film comprising a support having in order on one side thereof:

- (1) a radiation-sensitive layer comprising silver halide grains, a hydrophilic colloid and a polymer latex,
- (2) an interlayer consisting essentially of a hydrophilic colloid and a polymer latex, and
- (3) an overcoat layer consisting essentially of a hydrophilic colloid, a matting agent having an average particle size in the range of from about 1 to about 5 microns and a light-scattering agent having an average particle size in the range of from about 0.1 to about 5 microns; said interlayer having a refractive index in the range of from about 1.4 to about 1.7 and a thickness which is at least twice that of said overcoat layer and is in the range of from about 0.5 to about 5 microns.

2. A photographic film as claimed in claim 1 wherein said hydrophilic colloid in each of said radiation-sensitive layer, interlayer and overcoat layer is gelatin.

3. A photographic film as claimed in claim 1 wherein said interlayer has a thickness in the range of from about 0.8 to about 3.5 microns.

4. A photographic film as claimed in claim 1 wherein said interlayer has a thickness in the range of from about 1.7 to about 3 microns.

5. A photographic film as claimed in claim 1 wherein said overcoat layer has a thickness in the range of from about 0.2 to about 1 microns.

6. A photographic film as claimed in claim 1 wherein said polymer latex in said radiation-sensitive layer is present in an amount of from about 0.2 to about 1.5 parts per part by weight of said hydrophilic colloid in said radiation-sensitive layer.

7. A photographic film as claimed in claim 1 wherein said polymer latex in said interlayer is present in an

amount of from about 0.2 to about 1.5 parts per part by weight of said hydrophilic colloid in said interlayer.

8. A photographic film as claimed in claim 1 wherein said silver halide grains are doped with a doping agent, containing a nitrosyl or thionitrosyl coordination ligand and a transition metal of groups 5 to 10 of the periodic table of elements, in an amount sufficient to provide a level of photosensitivity which permits room-light-handling of said film.

9. A photographic film as claimed in claim 1 wherein said silver halide grains are doped with a doping agent in an amount sufficient to provide a level of photosensitivity which permits room-light-handling of said film, said doping agent being a transition metal coordination complex of the formula:



wherein

M is a ruthenium, rhenium, chromium, osmium or iridium transition metal,

X is oxygen or sulfur,

L is a ligand, and

n is —1, —2, or —3.

10. A photographic film as claimed in claim 1 wherein said matting agent is present in said overcoat layer in an amount of from about 0.02 to about 1 part per part by weight of said hydrophilic colloid in said overcoat layer.

11. A photographic film as claimed in claim 1 wherein said light-scattering agent is present in said overcoat layer in an amount of from about 0.02 to about 1 part per part by weight of said hydrophilic colloid in said overcoat layer.

12. A photographic film as claimed in claim 1 wherein the same material serves in said overcoat layer as both said matting agent and said light-scattering agent.

13. A photographic film as claimed in claim 1 wherein said matting agent is comprised of polymethyl methacrylate beads and said light-scattering agent is comprised of particles of silica.

14. A high-contrast room-light-handleable black-and-white silver halide photographic film which is especially adapted for use as a dry-dot-etchable contact film in the graphic arts by its ability to optically spread an image during contact exposure; said film comprising a support having in order on one side thereof:

- (1) a radiation-sensitive layer comprising gelatin, a polymer latex and silver halide grains doped with a doping agent in an amount sufficient to provide a level of photosensitivity which permits room-light-handling of said film, said doping agent being a transition metal coordination complex of the formula:



wherein M is a ruthenium, rhenium, chromium, osmium or iridium transition metal,

X is oxygen or sulfur,

L is a ligand and

n is —1, —2, or —3; and said radiation-sensitive layer having a thickness in the range of from about 2 to about 4 microns;

- (2) an interlayer consisting essentially of gelatin and a polymer latex and having a refractive index in the range of from about 1.55 to about 1.65 and a thick-

ness in the range of from about 1.7 to about 3 microns; and  
(3) an overcoat layer consisting essentially of gelatin, a matting agent, having an average particle size in the range of from about 1 to about 5 microns, and a light-scattering agent, having an average particle size in the range of from about 0.1 to about 5 microns, said overcoat layer having a thickness in the range of from about 0.3 to about 0.6 microns.

5

15. A photographic film as claimed in claim 14 wherein said doping agent is  $K_2Ru(NO)Br_5$ , said polymer latex in both said radiation-sensitive layer and said interlayer is poly(methylacrylate-co-2-acrylamido-2-methyl propane sulfonic acid), said matting agent consists of polymethyl methacrylate beads with an average size of 4 microns, and said light-scattering agent consists of particles of silica with an average size of 2 microns.

\* \* \* \* \*

10

15

20

25

30

35

40

45

50

55

60

65